

# UNITED STATES PATENT OFFICE.

HENRY LAVERS, OF SURREY HILLS, VICTORIA, AUSTRALIA, ASSIGNOR TO MINERALS  
SEPARATION AMERICAN SYNDICATE (1913) LIMITED, OF LONDON, ENGLAND.

## SEPARATION OF MIXED-SULFID ORES.

1,142,821.

Specification of Letters Patent. Patented June 15, 1915.

No Drawing.

Application filed May 28, 1914. Serial No. 841,477.

To all whom it may concern:

Be it known that I, HENRY LAVERS, a subject of the King of England, residing at Canterbury Road, Surrey Hills, State of Victoria, Australia, have invented certain new and useful Improvements in the Separation of Mixed Sulfid Ores, of which the following is a specification.

This invention relates to improvements in ore concentration and has for its object the separation of various metallic sulfids from each other by means of flotation separation. In this specification the word "ores" is intended to include concentrates, tailings, slimes or other products containing mixed metallic sulfids.

The present invention is a modification of that described in the previous United States Letters Patent to Greenway & Lowry No. 1,102,738 granted July 7, 1914. In that specification it is pointed out that if a salt of chromium (such as sodium bichromate or potassium bichromate) is introduced in solution into the circuit liquors in the agitation-froth process, or if the material to be treated is subjected to the action of such chromium salt solution by digestion or otherwise whereupon the material is subjected to flotation treatment, it is possible to obtain a flotation product relatively high in certain sulfids on the one hand and a residue relatively high in other sulfids on the other hand.

It is now found in treating finely pulverized material containing mixed sulfids particularly good results can be obtained if the pulp during digestion with the chromium salt in solution, and/or during flotation treatment with the chromium salt in solution, is slightly alkaline. For example the pulp may advantageously contain an amount of sodium carbonate equivalent to 1% by weight on the ore in the pulp.

A further feature of this invention is as follows: I have found that if the finely pulverized ore containing mixed sulfids and suspended in slightly alkaline water is subjected to the agitation-froth process with the use of a suitable frothing agent a flotation product can be obtained containing the bulk of the metallic sulfids which are thus separated from the gangue which mainly sinks. It is then found that if the concentrates be re-treated by the agitation-froth process (still in alkaline circuit) and with the addition of a salt of chromium, or after

digestion with such chromium salt solution, it is possible to obtain a flotation product relatively high in certain sulfids on the one hand and a residue relatively high in other sulfids on the other hand.

The following are examples of the application of this invention:

(1) An ore containing 9.0% of lead, 28.2% of zinc and 14.2% of iron, was very finely crushed and then subjected to froth-flotation treatment in apparatus of well-known type by being vigorously agitated with four times its weight of water at 130° F. containing in solution sodium carbonate amounting to about 22 lbs. per ton of ore, sodium bichromate amounting to about 6 lbs. per ton of ore, eucalyptus oil amounting to about  $\frac{1}{2}$  lb. per ton of ore and kerosene amounting to about  $\frac{1}{2}$  lb. per ton of ore. The flotation product obtained from this operation consisted of a concentrate containing 50.1% of zinc, 4.25% of lead and 8.3% of iron while the bulk of the iron and lead were left in the residue.

(2) Slimes containing about 11.6% of lead and 13.4% of zinc were introduced into an agitating apparatus together with four times their weight of water containing in solution carbonate of soda equivalent to 24 lbs. per ton of slimes to which was also added eucalyptus oil equivalent to about 1 lb. per ton of slimes at a temperature of about 130° F. The floating concentrate contained 22.2% of lead and 27.4% of zinc. The concentrate was then subjected to differential bichromate flotation, that is to say, the concentrate was subjected to flotation treatment of water at about 130° F. containing sodium carbonate equal to about 24 lbs. per ton of concentrate, sodium bichromate equal to 6 lbs. per ton of concentrate, kerosene equal to  $\frac{1}{2}$  lb. per ton of concentrate and eucalyptus oil equal to about  $\frac{1}{2}$  lb. per ton of concentrate. The flotation product contained 48.6% of zinc and 7.5% lead while the residue contained 8.9% zinc and 55.9% lead.

In most instances the action is facilitated by heating the solutions and I have found temperatures of from 120° F. to 150° F. to be in most cases suitable.

What I claim as my invention and desire to secure by Letters Patent is:

1. The herein-described process of concentrating metallic sulfid ores which consists

in subjecting the ore to the action of a chromium salt in a slightly alkaline solution and to a flotation separation whereby a flotation product relatively high in certain sulfids and a residue relatively high in other sulfids are obtained.

2. The herein-described process of concentrating metallic sulfid ores which consists in subjecting the ore to the action of a chromium salt in a slightly alkaline solution and to a flotation separation in a heated circuit whereby a flotation product relatively high in certain sulfids and a residue relatively high in other sulfids are obtained.

3. The herein-described process of concentrating metallic sulfid ores which consists in first crushing the ore to a suitable degree of fineness, then subjecting the crushed ore to a flotation separation in the presence of a solution of a salt of chromium and in a hot slightly alkaline circuit, whereby a flotation product relatively high in certain sulfids and a residue relatively high in other sulfids are obtained.

4. The herein-described process of concentrating metallic sulfid ores which consists in first crushing the ore to a suitable degree of fineness, then subjecting it to an agitation froth process of ore concentration in a slightly alkaline circuit for the formation of a froth containing the bulk of the metallic sulfids and thereafter subjecting the concentrate to a flotation separation treatment in the presence of a solution of a salt of chromium and in a slightly alkaline circuit whereby a flotation product relatively high in certain sulfids and a residue relatively high in other sulfids are obtained.

5. The herein-described process of concentrating ores containing zinc and lead sulfids consisting in first crushing the ore to a suitable degree of fineness, then subjecting the said ore to a flotation separation treatment in the presence of a solution of a

chromium salt and in a slightly alkaline circuit whereby there is obtained a flotation product relatively high in zinc and low in lead and a residue relatively high in lead and low in zinc.

6. The herein-described process of concentrating ores containing zinc and lead sulfids consisting in first crushing the ore to a suitable degree of fineness, then subjecting the said ores to a flotation separation treatment in the presence of a solution of bichromate of sodium and in a slightly alkaline circuit whereby there is produced a flotation product relatively high in zinc and low in lead and a residue relatively high in lead and low in zinc.

7. The herein-described process of concentrating ores containing zinc and lead sulfids consisting in first crushing the ore to a suitable degree of fineness, then subjecting the said ores to a flotation separation in the presence of a solution of sodium carbonate and bichromate of sodium whereby there is produced a flotation product relatively high in zinc and low in lead and a residue relatively high in lead and low in zinc.

8. The herein-described process of concentrating ores containing zinc and lead sulfids consisting in first crushing the ore to a suitable degree of fineness, then subjecting the said ores to a flotation separation in a hot circuit in the presence of a solution of sodium carbonate and bichromate of sodium whereby there is produced a flotation product relatively high in zinc and low in lead and a residue relatively high in lead and low in zinc.

In testimony whereof I have signed my name to this specification in the presence of two subscribing witnesses.

HENRY LAVERS.

Witnesses:

CHARLES NICHOLAS COLLISON,  
M. A. EUBLEY.